# EUROPEAN PATENT SPECIFICATION

(11) **EP 3 757 257 B1**
(45) Date of publication and mention of the grant of the patent: **16.08.2023**
(21) Application number: 20460020.9
(22) Date of filing: 27.04.2020
(51) Int. Cl.: C25D 11/02, C25D 11/26

(54) **THE FORMATION METHOD OF POROUS ANTIBACTERIAL COATINGS ON TITANIUM AND TITANIUM ALLOYS SURFACE**
VERFAHREN ZUR HERSTELLUNG VON PORÖSEN ANTIBAKTERIELLEN BESCHICHTUNGEN AUF DER OBERFLÄCHE VON TITAN UND TITANLEGIERUNGEN
PROCÉDÉ DE FORMATION DE REVÊTEMENTS ANTIBACTÉRIENS POREUX SUR UNE SURFACE DE TITANE ET D'ALLIAGES DE TITANE

(30) Priority: 25.06.2019 PL 43037519
(43) Date of publication of application: 30.12.2020
(73) Proprietor: Politechnika Slaska, 44-100 Gliwice (PL)
(72) Inventor: Simka, Wojciech, 40-748 Katowice (PL); Kazek-Kesik, Alicja, 41-310 Dabrowa Górnicza (PL); Lesniak, Katarzyna, 42-400 Zawiercie (PL)

(56) References cited:
- CN-A- 102 677 125
- PL-B1- 214 958
- KAZEK-KESIK ALICJA ET AL: "Surface characterisation of Ti-15Mo alloy modified by a PEO process in various suspens", MATERIALS SCIENCE AND ENGINEERING C, vol. 39, 12 March 2014 (2014-03-12), pages 259-272, XP029029210, ISSN: 0928-4931, DOI: 10.1016/J.MSEC.2014.03.008
- NECULA B S ET AL: "In vitro antibacterial activity of porous TiO"2-Ag composite layers against methicillin-resistant Staphylococcus aureus", ACTA BIOMATERIALIA, ELSEVIER, AMSTERDAM, NL, vol. 5, no. 9, 1 November 2009 (2009-11-01), pages 3573-3580, XP026693830, ISSN: 1742-7061, DOI: 10.1016/J.ACTBIO.2009.05.010 [retrieved on 2009-05-18]
- DATABASE EPODOC [Online] EUROPEAN PATENT OFFICE, THE HAGUE, NL; 20 May 1996 (1996-05-20), XP002800828, Database accession no. RU-94028190-A & RU 94 028 190 A (INST KHIM DAL NEVOSTOCHNOGO OTDEL RAN) 20 May 1996 (1996-05-20)
- MUHAFFEL FAIZ ET AL: "Characteristics of multi-layer coatings synthesized on Ti6Al4V alloy by micro-arc oxidation in silver nitrate added electrolytes", SURFACE AND COATINGS TECHNOLOGY, ELSEVIER BV, AMSTERDAM, NL, vol. 307, 1 September 2016 (2016-09-01), pages 308-315, XP029823815, ISSN: 0257-8972, DOI: 10.1016/J.SURFCOAT.2016.09.002

## Description

The subject of this invention is a formation method of the porous oxide layers on the surface of titanium and titanium alloys by plasma electrochemical oxidation. Due to the oxidation in baths containing suspended, insoluble particles of silver and copper compounds, the obtained oxide layers are intended to be characterized by antimicrobial and/or bacteriostatic properties.

Titanium and titanium alloys are used as long-term implant materials characterized by good biocompatibility with hard and soft tissue of the human body. During the implantation process, there is a risk of human tissues septic inflammation occurrence. Therefore, patients are being treated with bactericides such as antibiotics. However, because of the increasing resistance of bacteria to antibiotics, there are being carried out the studies of the alternative antibacterial agents. A good example of different than antibiotics bactericides can be the modified implant biomaterials containing silver or copper in their composition. So far in the literature, there are known studies of obtaining layers containing silver or copper compounds formed from soluble forms of these elements compounds.

The patent no. CN 101899700 describes the method of obtaining bioactive coatings on the surface of titanium and magnesium alloys by the plasma electrochemical oxidation using bath consisting of AgNO₃, which results in the formation of porous oxide layers containing calcium, phosphorus and silver improving the bioactivity of the coatings, as well as their corrosion resistance and decreasing the risk of bacterial infections caused by the implantation process. The thickness of the coating formed on the surface of the titanium alloy measured 50-85 µm, the porosity of the coating was in the range from 20% to 30%, and the determined adhesion of the coating to the substrate was 23-40 MPa. The patent no. CN 108543109 describes the formation method of composite materials with antibacterial properties. The composite consists of ceramic TiO₂ and silver nanoparticles on the surface of a titanium alloy intended for use as an implant for bone tissue. In the paper "Antibacterial properties of Ag (or Pt)-containing calcium phosphate coatings formed by micro-arc oxidation" (W.H. Song, H.S. Ryu, S.H. Hong, Journal of Biomedical Materials Research Part A, 88 (1) (2009) 246) there is known the method of plasma electrochemical oxidation using the bath containing: 0.04 mol·dm⁻³ C₃H₇Na₂O₆P·5H₂O, 0.40 mol·dm⁻³ (CH₃COO)₂Ca·H₂O and AgNO₃ or CH₃COOAg in the concentration range 0.00003-0.004 mol·dm⁻³ at 250-450 V. The manuscript "Antibacterial titanium surfaces for medical implants" (S. Ferraris, S. Spriano, Materials Science and Engineering, 61 (2016) 965) presents the method of plasma electrochemical oxidation using a bath containing 7-25 nm silver nanoparticles, (CH₃COO)₂Ca and calcium glycerophosphate. The paper "Fabrication of oxide layer on zirconium by micro-arc oxidation: Structural and antimicrobial characteristics" (S. Fidan, F. Muhaffel, M. Riool, G. Cempura, L. de Boer, S. A. J Zaat, A. Czyrska- Filemonowicz, H. Cimenoglu, Materials Science and Engineering, 71 (2017) 565) presents the method of plasma electrochemical oxidation using the bath containing Na₂SiO₃, NaOH and CH₃COOAg. In the manuscript "Characteristics of multi-layer coatings synthesized on Ti6Al4V alloy by micro-arc oxidation in silver nitrate added electrolytes" (F. Muhaffel, G. Cempura, M. Menekse, A. Czyrska-Filemonowicz, N. Karaguler, H. Cimenoglu, Surface and Coating Technology. 307 (2016) 308) there is known the method of plasma electrochemical oxidation in the bath containing Na₂HPO₄, Ca(CH₃COO)₂·H₂O and AgNO₃ in concentrations 0.1 g·dm⁻³ or 0.4 g·dm⁻³. In the manuscript "Corrosion Resistance and Antibacterial Properties of Ag-Containing MAO Coatings on AZ31 Magnesium Alloy Formed by Microarc Oxidation" (S. Ryu, SH Hong, Journal of Electrochemical Society, 157 (2010) 131), the method of plasma electrochemical oxidation in bath containing Na₂SiO₃ and AgNO₃ is known. The paper "High-current anodization: A novel strategy to functionalize titanium-based biomaterials" (C. Chang, X. Huang, Y. Liu, L. Bai, X. Yang, R. Hang, B. Tang, PK Chu, Electrochimica Acta, 173 (2015) 345) presents the method of plasma electrochemical oxidation in the bath containing 7.6 g·dm⁻³ Na₃PO₄, 9.4 g·dm⁻³ Ca(NO₃)₂ and 1.0 g·dm⁻³ AgNO₃. The publication "In vitro antibacterial activity of porous TiO2-Ag composite layers against methicillin-resistant Staphylococcus ureus" (B.S. Necula, L.E. Fratila-Apachitei, S.A. Zaat, I. Apachitei, J. Duszczyk, Acta Biomaterialia, 5 (2009) 3573) presents the method of plasma electrochemical oxidation in the bath containing 0.15 mol·dm⁻³ Ca(CH₃COO)₂ or 0.02 mol·dm⁻³ calcium glycerophosphate with the addition of 0.03 g·dm⁻³ of nanoparticles Ag. The manuscript "Characteristics of multi-layer coating formed on commercially pure titanium for biomedical applications" (D. Teker, F. Muhaffel, M. Menekse, NG Karaguler, M. Baydogan, H. Cimenoglu, Materials Science and Engineering C, 48 (2015) 579) presents the method of anodic electrochemical oxidation using the bath containing Na₂HPO₄, Ca(CH₃COO)₂ and 0.0025 mol·dm⁻³ CH₃COOAg. In the paper "Corrosion behavior of Zn-incorporated antibacterial TiO2 porous coating on titanium" (X. Zhang, H. Wang, J. Li, X. He, R. Hang, X. Huang, L. Tian, B. Tang, Ceramic International, 32 (2016) 919) there is presented the method of anodic electrochemical oxidation in the bath consisting of 0.02 mol·dm⁻³ sodium β-glycerophosphate, 0.1 mol·dm⁻³ Ca(CH₃COO)₂, 0.1 mol·dm⁻³ Zn(CH₃COO)₂ and 6 g·dm⁻³ of nanoparticles Ag. In the manuscript "Energy-Dispersive X-Ray Spectroscopy Mapping of Porous Coatings Obtained on Titanium by Plasma Electrolytic Oxidation in a Solution Containing Concentrated Phosphoric Acid with Copper Nitrate" (K. Rokosz, T. Hryniewicz, L. Dudek, A. Schutz, J. Heeg and M. Wienecke, Advances in Materials Science, 16 (2016) 15) there is presented the method of anodic oxidation of titanium using the bath containing Cu(NO₃)₂. 1 dm³ of bath may contain 85% H₃PO₄ and 600 g of dissolved Cu(NO₃)₂. The process can be carried out at 450 V. In the work "Catalytically active cobalt-copper-oxide layers on aluminium and titanium" (I.V. Lukiyanchuk, I.V. Chernykh, V.S. Rudnev, A. Yu Ustinov, L.M. Tyrina, P.M. Nedozorov, E.E. Dmitrieva, Protection of Metals and Physical Chemistry of Surfaces, 50 (2014) 209) there is known the method of obtaining oxide layers on the titanium surface by the plasma electrolytic oxidation treatment, followed by the modification of the obtained oxide layers with copper and cobalt by impregnation in solutions of soluble copper and cobalt salts. The manuscript "Biological Activity and Antibacterial Property of Nano-structured TiO2 Coating Incorporated with Cu Prepared by Micro-arc Oxidation" (W. Zhu, Z. Zhang, B. Gu, J. Sun, L. Zhu, Journal of Materials Science & Technology, 29 (2013) 237) a plasma electrochemical oxidation method is known using the bath containing 0.05 mol-dm' ³ sodium β-glycerophosphate, 0.1 mol·dm⁻³ Ca(CH₃COO)₂ and 0.05 mol·dm⁻³ (CH₃COO)₂Cu. The publication "SEM, EDS and XPS Analysis of the Coatings Obtained on Titanium after Plasma Electrolytic Oxidation in Electrolytes Containing Copper Nitrate" (K. Rokosz, T. Hryniewicz, D. Matysek, S. Raaen, J. Valí ek, . Dudek, M. Harni árová, Materials, 9 (2016) 318) describes the method of anodic oxidation of titanium from the bath containing Cu(NO₃)₂. 1 dm³ of bath may contain 85% H₃PO₄ and 10-600 g of dissolved Cu(NO₃)₂. In the paper "Microstructure and antibacterial properties of Cu-doped TiO2 coating on titanium by micro-arc oxidation" (X. Yao, X. Zhang, H. Wu, L. Tian, Y. Ma, B. Tang, Applied Surface Science , 292 (2014) 944) there is known the method of plasma electrochemical oxidation in the bath containing 2 g·dm⁻³ NaOH, 15 g·dm⁻³ NaH₂PO₄ and 3 g·dm⁻³ Cu nanoparticles. In the manuscript "One-step fabrication of cytocompatible micro/nano-textured surface with TiO₂ mesoporous arrays on titanium by high current anodization" (X. Huang, Y. Liu, H. Yu, X. Yang, Y. Wang, R. Hang, B. Tang, Electrochimica Acta, 199 (2016) 116) there is known the method of anodic electrochemical oxidation using the bath containing 3.8-7.6 g·dm⁻³ Na₃PO₄ and 1.0-8.0 g·dm⁻³ Cu(NO₃)₂. The paper "The dual function of Cu-doped TiO2 coatings on titanium for application in percutaneous implants" (L. Zhang, J. Guo, X. Huang, Y. Zhang, Y. Han, Journal of Materials Chemistry, 4 (2016 ) 3788) presents the method of anodic electrochemical oxidation using the bath containing 0.02 mol·dm⁻³ sodium β-glycerophosphate, 0.02 mol·dm⁻³ Ca(CH₃COO)₂ and 0.00125-0.00500 mol·dm⁻³ Cu(CH₃COO)₂. The patents No. PL 225226 and PL 225227 present the method of anodic electrochemical oxidation of tantalum, niobium and zirconium in the suspension of insoluble calcium silicate CaSiO₃ at a concentration of 1-300 g·dm⁻³.

The patent no. PL 396115 present the method of plasma electrochemical oxidation of titanium and its alloys in suspension ZrSiO₄ at a concentration of 1-100 g·dm⁻³ with the addition of an alkali metal hydroxide at a concentration of 5-100 g·dm⁻³, temperature of 15-50°C, anodic current density 5-500 mA·dm⁻² and applied voltage 1-600 V for 1-30 minutes. In the patent no. PL 214630 there is presented the method of electrochemical plasma oxidation of Ti-xNb-yZr alloys in a Ca(H₂PO₂)₂ solution at a concentration of 1-150 g·dm⁻³ or in a NaH₂PO₂ solution at a concentration of 1-250 g·dm⁻³, temperature in the range of 15-50°C, anodic current density of 5-5000 mA·dm⁻² and applied voltage of 100-650 V for 1-60 minutes.

The paper "Surface characterisation of Ti-15Mo alloy modified by a PEO process in various suspensions" (A.Kazek-K sik, G. Dercz, I. Kalemba, K. Suchanek, A. Kukharenko, D. Korotin, J. Michalska, A. Krz ka a, J.Piotrowski, E. Kurmaev, S. Cholakh, W. Simka, Materials science and engineering, vol.39 (2014)) reports on the surface modification of a Ti-15Mo alloy by plasma electrolytic oxidation (PEO). This process was carried out in solutions of 0.1M Ca(H2PO2)2 with various concentrations of tricalcium phosphate (Ca3(PO4)2), wollastonite (CaSiO3), or silica (SiO2) using voltages of up to 350V. The surface microstructure (SEM, cross-section of coating), roughness and chemical composition (energy-dispersive X-ray spectroscopy, thin layer X-ray diffraction, X-ray photoelectron spectroscopy and Raman spectroscopy) of the porous oxide layers were investigated. The concentration of powder added to the solution changed the chemical composition and morphology of PEO coatings on the Ti-15Mo alloy surface. Calcium and phosphorous compounds were detected in the coatings formed on the substrate by the PEO process at 300V.

The aim of the invention is to develop a method allowing to obtain the porous oxide layers with incorporated compounds with antibacterial properties.
The essence of the invention is the surface modification by plasma electrochemical oxidation in aqueous Ca(H₂PO₂)₂ bath at the concentration from 0.01 mol·dm⁻³ to 5 mol·dm⁻³ with the anodic current density from 1 mA·cm⁻² to 250 mA·cm⁻² and applied voltage from 50 V to 600 V by immersing the element which surface is to be modified in the aqueous Ca(H₂PO₂)₂ bath solution characterized in that the bath comprises insoluble particles of silver(I) oxide Ag₂O, copper(I) oxide Cu₂O or copper(II) oxide CuO at a concentration from 1 g·dm⁻³ to 400 g·dm⁻³.

The invention describes the method of the plasma electrochemical oxidation of titanium and its titanium alloys in suspensions containing insoluble silver or copper compounds in the form of the oxides. In this way, it is possible to obtain porous oxide layers incorporated with particles of compounds characterised by the antibacterial properties. The addition of mentioned silver and copper suspension compounds can be a one-step modification of the surface of titanium and its alloys. Thanks to this, there is a chance to eliminate the necessity of high, oral antibiotic delivery route, which is the main cause of increasing bacteria resistance to antibiotics. Additionally, the number of side effects and allergic reactions related to antibiotic treatment can be reduced. The surfaces anodised via plasma electrolytic oxidation process are porous and rough, which promotes the proliferation of living cells and supports the osseointegration process.

Example 1: The titanium implant, pre-treated by polishing, degreasing, etching and rinsing in demineralised water is placed in the solution containing 0.1 mol·dm⁻³ Ca(H₂PO₂)₂ and the suspension of 10 g·dm⁻³ Ag₂O. After placing the implant in the anodising bath, the electrolytic plasma oxidation process is carried out by polarizing it with the anodic current density of 150 mA·cm⁻². The process is carried out for 5 minutes, with the maximum voltage of 300 V. After the process, the implant is rinsed in demineralised water and air-dried at 45°C.

Example II: The implant made of Ti-13Nb-13Zr alloy, mechanically pre-treated, degreased, etched and rinsed in demineralised water is placed in the anodising bath containing 0.01 mol·dm⁻³ Ca(H₂PO₂)₂ and a suspension of 100 g·dm⁻³ Cu₂O. After placing the implant in the bath, the electrolytic plasma oxidation process is carried out by polarizing it with the anodic current density of 100 mA·cm⁻². The process is carried out for 7 minutes, with the maximum voltage of 350 V. After the process, the implant is rinsed in demineralised water and air-dried at 45°C.

Example III: The implant made of Ti-15Mo alloy, mechanically pre-treated, degreased, etched and rinsed in demineralised water is placed in the anodising bath containing 5 mol·dm⁻³ Ca(H₂PO₂)₂ and the suspension of 200 g·dm⁻³ CuO. After placing the implant in the bath, the electrolytic plasma oxidation process is carried out by polarizing it with the anodic current density of 200 mA·cm⁻². The process is carried out for 5 minutes, with the maximum voltage of 400 V. After the process, the implant is rinsed in demineralised water and air-dried at 45°C.

## Claims

1. The method of titanium surface modification by plasma electrochemical oxidation in aqueous Ca(H₂PO₂)₂ bath at the concentration from 0.01 mol·dm⁻³ to 5 mol·dm⁻³ with the anodic current density from 1 mA·cm⁻² to 250 mA·cm⁻² and applied voltage from 50 V to 600 V by immersing the element which surface is to be modified in the aqueous Ca(H₂PO₂)₂ bath solution **characterized in that** the bath comprises insoluble particles of silver(I) oxide Ag₂O, copper(I) oxide Cu₂O or copper(II) oxide CuO at a concentration from 1 g·dm⁻³ to 400 g·dm⁻³.

## Patentansprüche

1. Das Verfahren zur Oberflächenmodifikation von Titan durch plasmaelektrochemische Oxidation in einem wässrigen Ca(H₂PO₂)₂ Bad mit einer Konzentration von 0,01 mol/dm⁻³ bis 5 mol/dm⁻³, einer anodischen Stromdichte von 1 mA/cm⁻² bis 250 mA/cm⁻² und einer angelegten Spannung von 50 V bis 600 V, indem das Element, dessen Oberfläche modifiziert werden soll, in der wässrigen Ca(H₂PO₂)₂-Badlösung eingetaucht wird, **gekennzeichnet dadurch, dass** das Bad unlösliche Partikel von Silber(I)-oxid Ag₂O, Kupfer(I)-oxid Cu₂O oder Kupfer(II)-oxid CuO in einer Konzentration von 1 g/dm⁻³ bis 400 g/dm⁻³ enthält.

## Revendications

1. La méthode de modification de la surface du titane par oxydation électrochimique par plasma dans un bain aqueux de Ca(H₂PO₂)₂ à une concentration de 0.01 mol-dm⁻³ à 5 mol dm⁻³ avec une densité de courant anodique de 1 mA cm⁻² à 250 mA cm⁻² et une tension appliquée de 50 V à 600 V en immergeant l'élément dont la surface doit être modifiée dans la solution aqueuse du bain de Ca(H₂PO₂)₂ **caractérisée par le fait que** le bain comprend des particules insolubles d'oxyde d'argent (I) Ag₂O, d'oxyde de cuivre (1) Cu₂O ou d'oxyde de cuivre (II) CuO à une concentration de 1 g dm⁻³ à 400 g dm⁻³.
